

Patented May 1, 1928.

1,668,307

## UNITED STATES PATENT OFFICE.

JOSEPH G. DONALDSON AND HENRY L. COLES, OF HAMILTON, OHIO, ASSIGNEES TO  
GUARDIAN METALS COMPANY, OF HAMILTON, OHIO, A CORPORATION OF DELA-  
WARE.

## ALLOY AND MATERIAL EMPLOYING THE SAME.

No Drawing.

Application filed May 19, 1923. Serial No. 640,226.

Our invention, although not limited thereto, concerns more particularly material, such as safe and vault plates and the like, adapted to resist attack by the local application of high heat, as by means of the oxy-acetylene torch. It has long been known that copper, because of its high heat conductivity and the fact that it cannot be cut by oxidation, offers substantial resistance to penetration by means of high heat locally applied. It has been found defective, however, for the reason that its melting point is relatively low and also because it flows freely when it has been brought to a melting temperature. We have found a way to raise the melting point of copper and, at the same time, preserve or increase its high heat conductivity and also to produce a material which does not flow when brought to a melting temperature as by the local application of high heat. We accomplish these results by the addition to copper of relatively small amounts of silicon and carbon, it having been found that such addition profoundly affects the physical qualities of the copper, producing a material having the characteristics above stated. A typical formula of such an alloy would be approximately as follows, disregarding the impurities commonly found in refined copper, such as small amounts of iron, lead and tin, which may be present without serious detriment thereto:—

|         | Per cent.        |
|---------|------------------|
| Silicon | .60 to .75       |
| Carbon  | .015 to .020     |
| Copper  | 99.385 to 99.230 |

In carrying out our invention, the copper is first made molten, preferably in a direct-arc type electric furnace. If other means are employed for melting, then carbon should be added to the copper during the time of the melting, thereby assisting in the process of deoxidation thereof. If the metal is heated in a direct-arc type electric furnace, then it is not necessary to add a separate portion of carbon to the mixture, inasmuch as this ingredient will be furnished by the drippings from the electrodes. After the metal has been brought to a high heat, we add thereto from 2 to 2½% by weight of 30% cupro-

silicon in powdered form. The alloying takes place very quickly with much loss of heat and a notable change takes place in the color of the molten metal. It is necessary to stir the metal rapidly; otherwise, this alloying will be largely a surface phenomenon and the surface of the molten bath will tend to freeze. After the metals are thoroughly mixed, the alloy can be poured in the regular way, as by means of a ladle. As an alternative, the cupro-silicon can be made molten and can be mixed with the copper while the latter is either in the furnace or the ladle.

The resulting alloy resists best when the silicon content is from .60 to .75%. If greater or less amounts of silicon are added, there is a notable change in the resistance of the metal. If too great an amount of silicon is added, then the resistance of the alloy becomes less than that of copper.

In a previous application we have described material characterized by a core having a high-melting point encompassed by another metal, termed by us the "sheath" metal, preferably having high heat conductivity. The alloy disclosed above makes an excellent "sheath" metal, inasmuch as it cannot be cut by oxidation and yields very slowly when extremely high heat is locally applied. As pointed out above, this alloy will not flow when raised above its melting point but appears to slowly slough off in very small flakes.

Another method of utilizing this alloy is to use the same as a "core" and to encompass the alloy in other metal, such as cast iron, steel and the like. Here the core and sheath will be rigidly united, the areas in contact being, in fact, alloys of the core and sheath materials. On account of its very high heat conductivity and its other peculiar properties, it has been found that such a core will resist prolonged attacks by means of the oxy-acetylene torch. The encompassing of this alloy in another metal permits its use in much thinner strata. Tests have shown that these are impenetrable to the torch, notwithstanding the fact that the same thickness of the alloy not so encompassed is penetrated with relative ease. It has also been found

that an alloy of copper and silicon is superior to copper and other non-ferrous metals when used either as a sheath metal as described above, or as a core encompassed by 5 other metals.

When using the alloy herein described as a core, we may combine another metal (as cast-iron) therewith and then encompass the whole in a suitable sheath metal such as 10 steel. In such case, the alloy may form from 15 to 30 per cent of the core.

So-called torch-resisting plates have heretofore been suggested in which copper and cast iron in varied proportions have been 15 combined. The best results can be obtained in such plates when the copper content is approximately 20 to 25% of the entire mixture. Plates so constructed, however, may be melted when attacked by means of the 20 largest size torches. The cast iron will absorb only about 5% of the copper and the remaining copper is, therefore, unequally distributed throughout the mass, the cast iron constituting the matrix in which the 25 excess copper is embedded. Our new alloy, however, employed as above stated, greatly increases the resistance of the plate to attack in the forms herein suggested.

Having now described our invention, what

we claim and desire to secure by Letters 30 Patent is as follows:—

1. A compound plate consisting of a core which is an alloy of 99.385-99.230% copper, .015-.020% carbon and .60-.75% silicon, said core being encompassed by other metal 35 and united thereto as by alloying therewith.

2. A new article of manufacture being the combination of a plate of an alloy of a majority portion of copper, carbon, and silicon between .60-.75%, which alloy may be penetrated by a torch when taken alone, and a high melting point metal joined to said alloy plate to form a compound plate that is 40 not penetrable by the torch.

3. A substantially integral metallic structure, comprising a metal having a high melting point, and an alloy of copper, less than .75% silicon and less than .015% carbon, said structure being resistant to local high 45 heat as produced by an acetylene cutting blow torch.

4. A plate consisting of cast iron surrounding an alloy of 99.385-99.230% copper, .60-.75% silicon, and .015-.020% carbon.

This specification signed this 16 day of 55 May, 1923.

JOSEPH G. DONALDSON.  
HENRY L. COLES.